

## UNITED STATES PATENT OFFICE

2,178,791

## PICKLING OF STEEL

Donald Cleve Hilty, Apollo, Pa.

No Drawing. Application December 29, 1937,  
Serial No. 182,321

2 Claims. (Cl. 148—8)

This invention relates to the pickling of steel and is particularly concerned with the removal of red oxide from silicon steel. In explanation, silicon steel sheets, upon being annealed, develop 5 a reddish surface color in addition to the usual scale to be expected. Ordinary pickling does not remove this red color.

According to the present invention, a pickling bath is prepared which contains, in addition to 10 the usual concentration of sulphuric acid, sulphur dioxide to the extent of at least .025 per cent. by weight of the solution. In some instances hydrochloric acid may be added to accelerate the scale removal. Other pickling 15 additions may be made, such as that of the various inhibitors which have become common. In case it is desired to remove the reddish color without also removing the scale, the acid concentration may be kept to a very low value, bleaching 20 occurring if the sulphur dioxide concentration is above the factor mentioned.

The objectionable reddish tinge is removed from annealed silicon sheets upon immersion in either of the above solutions. In the case of a 25 solution having a normal acid concentration common to pickling liquors, both the reddish color and ordinary scale will be removed. In the case of certain types of silicon sheets the scale remains, and in such instances the solution containing 30 a low concentration of acid but including the sulphur dioxide functions to bleach the reddish color to a uniform grayish tint. It has been found that here is an abrupt decrease in the solubility of sulphur dioxide gas in acid pickling solution as the temperature of the solution is raised 35 above 140 degrees Fahrenheit.

As a specific example, the removal of both ordinary scale and red oxide from annealed silicon steel sheets may be effected by immersing the 40 sheets for ten minutes in an ordinary 7 per cent, sulphuric acid pickling solution containing, however, .025 per cent. or more by weight of sulphur dioxide, with the solution at a temperature not exceeding 140 degrees Fahrenheit. The scale re-

moving action of the solution may be accelerated by the addition of a small amount of hydrochloric acid. The sulphur dioxide concentration may be maintained by direct injection of the gas or by the use of suitable compounds which release this 5 gas upon reaction with the pickling solution. Examples of such compounds are sodium sulphite, sodium bi-sulphite, or sodium thiosulphate.

In case bleaching alone is desired the pickling solution used should not contain more than 1.0 10 per cent. by weight of sulphuric acid. No hydrochloric acid should be used. Immersion of the sheets for five minutes at a temperature of 140 degrees Fahrenheit in such a pickling solution including, of course, the proper concentration of 15 sulphur dioxide, will remove the red color without materially affecting the normal scale. Preferably, a suitable inhibitor should be added to the solution.

I claim:

20

1. A process of removing the red color from heat treated silicon steel without substantial scale removal, including subjecting the steel to the action of a slightly acid solution containing sulphur dioxide while maintaining the solution 25 at temperatures not exceeding 140 degrees Fahrenheit, the sulphur dioxide being maintained at a concentration sufficient to effect removal of the red color and the acidity of the solution being sufficiently low to prevent substantial scale 30 removal.

2. A process of removing the red color from heat treated silicon steel without substantial scale removal, including subjecting the steel to the action of a slightly acid solution containing 35 sulphur dioxide while maintaining the solution at temperatures not exceeding 140 degrees Fahrenheit, the sulphur dioxide being maintained at a concentration in excess of .025 per cent by weight of the solution to effect removal of the red color 40 and the acidity of the solution being sufficiently low to prevent substantial scale removal.

DONALD CLEVE HILTY.